

April 18, 1967

J. M. PERRI

3,314,845

METHOD OF FLOCKING AND SUBSEQUENTLY DEVELOPING LATENTLY  
CRIMPABLE FIBERS AND ARTICLE PRODUCED THEREBY  
Filed July 23, 1964

2 Sheets-Sheet 1



INVENTOR  
JOSEPH MARK PERRI

BY

*Donald A. Hoer*

ATTORNEY

April 18, 1967

J. M. PERRI

3,314,845

METHOD OF FLOCKING AND SUBSEQUENTLY DEVELOPING LATENTLY  
CRIMPABLE FIBERS AND ARTICLE PRODUCED THEREBY

Filed July 23, 1964

2 Sheets-Sheet 2

FIG. 3



INVENTOR  
JOSEPH MARK PERRI

BY

*Donald A. Osses*  
ATTORNEY

# United States Patent Office

3,314,845

Patented Apr. 18, 1967

1

3,314,845  
METHOD OF FLOCKING AND SUBSEQUENTLY  
DEVELOPING LATENTLY CRIMPABLE FIBERS  
AND ARTICLE PRODUCED THEREBY  
Joseph Mark Perri, Waynesboro, Va., assignor to E. I. du  
Pont de Nemours and Company, Wilmington, Del., a  
corporation of Delaware  
Filed July 23, 1964, Ser. No. 384,647  
16 Claims. (Cl. 161—64)

This application is a continuation-in-part of copending application Serial No. 302,713, filed August 16, 1963, now abandoned.

This invention relates to novel pile fabrics of improved aesthetic appeal and outstanding functional properties and to a flocking process useful for obtaining such fabrics.

Flocking techniques involving the application of staple fibers to an adhesive coated backing have been practiced commercially for many years in the manufacture of a wide variety of products. The majority of these techniques have, however, been restricted to the utilization of short straight fibers owing to certain inherent limitations in the electrostatic depositing processes which are commonly employed for that purpose; i.e., crimped and curved fibers cannot be readily propelled against a backing to give an ordered assembly. Although such techniques have more recently been successfully adapted to the production of carpets and related structures by flocking of short straight synthetic fibers, e.g. nylon fibers, the resultant products, while often possessing good wear-resisting properties, have been characterized by several attendant disadvantages. Thus the attainment of a wide range of pile heights for such carpets has been severely limited owing to the relatively short lengths of nylon fibers which can be satisfactorily flocked on a commercial scale. In addition, the pile density of typical carpets so produced has been relatively low such that the products have a "lean" appearance and hence possess poor cover. Still a further disadvantage has been that sustained loads upon the surface of the carpets give rise to imprints which are not readily removed due to the inability of the compressed straight fibers to recover their original position upon removal of the applied force.

Accordingly it is an object of the invention to provide a novel process for preparing flock pile fabrics. An additional object is the attainment of pile fabrics having a superior combination of properties in comparison with flocked fabrics which have heretofore been available. Another object is to provide fabrics having a superior cover and which are composed of synthetic pile fibers. A further object is to provide an improved flocking process for preparing superior suedes, velvets, carpets, furs, blankets, and laminated insulating fabrics. Other objects will be apparent from the description of the invention given below.

In accordance with the present invention there is provided a method for the manufacture of pile fabrics comprising the steps of providing a plurality of short straight, latently crimpable synthetic organic polymeric fibers which have been treated to temporarily inhibit premature crimp, depositing the thusly treated fibers upon an adhesive coated backing material to provide a pile layer of upstanding fibers thereon, and treating the resultant fabric to develop the latent crimpability of the fibers.

By the term "latently crimpable" as used herein to describe the fibrous starting material, it is meant that although the fibers be in a generally straight condition they nevertheless possess an inherent tendency to take on or otherwise assume an irregular contorted configuration by exposure thereof to heat, moisture or other chemicals, or by a combination thereof, without the exertion of a

2

mechanical force upon the fibers to disrupt the otherwise generally straight condition. It is essential that the fibers be capable of not merely assuming a generally curved or flexed shape but, rather, that they be capable of affording a crimp frequency of at least about 1 crimp per inch as well as a minimum crimp index of 10%.

The crimp index is a measure of the amount of crimp in that it designates the difference in length between a fiber in crimped and in uncrimped (or extended) condition as expressed as a percentage of the uncrimped length.

The novel pile fabrics of the invention, advantageously derived as products of the above described process, possess an advantageous combination of properties including high bulk and excellent compressional properties and cover. These pile fabrics comprise a plurality of short synthetic organic polymeric fibers individually and randomly attached in generally upstanding relationship to an adhesive layer, the pile formed of said fibers comprising a support portion occupied by the lower 50% sections of the extended length of said fibers and an upper portion occupied by the remaining 50% sections of the extended length of said fibers, fiber sections in said support portion being essentially spaced apart, free of crimp, and perpendicularly aligned with respect to said adhesive layer, fiber sections in said upper portion having an average crimp frequency of 1 to 8 crimps per inch thereby creating a pile surface having a random and multi-directional array of fiber sections and fiber-to-fiber entanglements. These novel pile fabrics will be described in further detail below in connection with the drawings.

In the above defined pile fabrics the crimped section of the fibers will be seen to possess a curved or curled configuration. In other words such a fiber will trace a bend or gradual change in direction, e.g. as shown in FIGURES 1 and 2, as opposed to many types of mechanically crimped fibers which exhibit an abrupt change in direction, e.g. the well known stuffer-box or saw-tooth crimped configuration. Because the flock fibers are of a relatively short length and have one end permanently fixed in the adhesive layer, upon development of the crimp they are not able to develop a full helical configuration but for the most part will be simply two dimensional. As is well known, fibers which have a latent capacity to crimp, for example bicomponent fibers, if caused to crimp without external restraint, will tend to take on a helical configuration.

The term "crimp frequency" as employed herein is a measure of the relative curvature existing in the crimped section of the fiber in the pile fabric. Because the crimped section will normally trace only a portion of the closed circle, direct counting of the number of crimp reversals in the ordinary fashion would have no significance. For purposes of the present invention crimp frequency is conveniently obtained as a function of the circumference of a circle that the major arc of the crimped section of the fiber would trace if extended, specifically

$$\text{crimp frequency} = \frac{1}{\text{circumference}} = \frac{1}{2\pi \cdot \text{radius}}$$

The fibrous starting materials employed in the process of the invention are short straight, latently crimpable, synthetic organic polymeric fibers. For most purposes a suitable flocking length for the straight fibers is about 0.01 to 0.5 inch, although more commonly fibers will be employed which have a length of about 0.1 to 0.35 inch. The fibers will be composed of either linear condensation polymers or linear addition polymers, for example, acrylonitrile polymers and copolymers; polyamides, such as polyhexamethylene adipamide, polycaproamide, poly-(meta-phenylene isophthalamide), and copolyamides; polyesters such as polypivalolactone, polyethylene terephthal-

ate and copolymers prepared from glycols and terephthalic and isophthalic acids; polyethylene and ethylene copolymers; polypropylene and propylene copolymers; polybenzimidazole; copolymers of acrylonitrile with small amounts of copolymerizable monomers (e.g. with 12% by weight methyl methacrylate or with 10% by weight vinyl acetate); and the like. Each of the synthetic fibers selected for use in accordance with the invention must be prepared under conditions such that a latent capacity to crimp is built into the fiber. Suitable techniques for preparing fibers with latent crimp are described in the following U.S. patents and applications: Sisson 2,439,815, Taylor 3,038,237, Breen 3,038,236, Zimmerman 3,038,235, Moulds 3,038,239, Kilian 3,050,821, Hebler 2,604,689, and Olson Serial No. 335,187, filed Jan. 2, 1964. The fibers disclosed in those patents and the application are well suited to the practice of the instant invention.

One suitable fiber having a latent capacity to crimp is a bicomponent acrylic fiber wherein one component of the fiber is composed of polyacrylonitrile and the other component is composed of a copolymer of acrylonitrile with 6 to 20% by weight of vinyl acetate.

A particularly suitable class of short straight, latently crimpable, synthetic organic polymeric fibers can be prepared by cutting short fibers from the composite filaments described and claimed in aforementioned Taylor U.S. Patent 3,038,237. Among the multi-component fibers described in that patent, a preferred class is represented by those in which each of the two or more components is composed of at least 85% by weight of recurring units derived from acrylonitrile. Especially suitable pile fibers are composed of a bicomponent acrylonitrile polymer fiber in which one side of the fiber is composed of polyacrylonitrile and the other side of the fiber is composed of a copolymer of acrylonitrile with between 1% and 5% of sodium styrene sulfonate. The latent crimpability attributed to the multicomponent fibers of that patent results from the co-spinning, side by side, of two or more selected synthetic materials differing in ionizable content.

In flocking fibers upon an adhesive coated substrate it is important to the achievement of satisfactory appearance and performance properties that the fibers be disposed in an upstanding or generally perpendicular relationship with respect to the substrate. For this reason it is essential that the fibers initially possess a generally straight extended configuration and that such configuration be maintained during the flocking process. Since the flock fibers employed in accordance with the invention have a latent capacity to crimp, it is furthermore essential that they do not become prematurely crimped prior to upstanding adherence to the backing. To temporarily inhibit such undesirable deviation from the essentially straight condition it is necessary to appropriately treat the fibers, e.g. to rigidify the fibers in a temporary state which can be later removed or otherwise destroyed following the flocking step. The crimp inhibition means may be, for example, a simple operation wherein after spinning, drawing and any subsequent hot wet treatment, the fibers are held tautly in the lengthwise dimension and dried. Of course, fibers may be spun and collected in a normal manner followed at a later time by remoistening and drying in a taut condition. Alternatively the fibers may be coated with 10% by weight or more of a water-repellent weighting agent, such as paraffin wax or a chlorinated wax.

Because synthetic organic polymeric fibers are normally non-conductive, it is especially desirable that they be treated prior to flocking with an antistatic agent. As is well known in the art the antistatic agents function by imparting a hydrophilic property hence electrical conductivity, to the surface of the synthetic fibers, most of which are relatively hydrophobic in nature. Both ionic and non-ionic substances and mixtures thereof are commonly em-

ployed for reducing the static attractive forces. Typical antistatic agents which are suitable for treating fibers prior to flocking in accordance with the invention include the condensation products of ethylene oxide with alkyl phenols, e.g. nonyl phenol, or fatty acids, e.g. of 12 to 18 atoms. Such products commonly contain between 20 and 90% by weight of ethylene oxide. Other suitable antistatic agents include the pyrophosphonate condensation products of phosphorus pentoxide and fatty acids of 12 to 18 carbon atoms, combinations of the latter acids with cetyl trimethyl ammonium bromide, and triethanolamine oleate.

Since the antistatic agents are usually water soluble and hygroscopic, normally it will be highly desirable to use a so-called "separating agent" to treat the fibers prior to flocking. The separating agents can be particulate solids which serve to reduce fiber-to-fiber adhesion; that is, they keep the fibers individually suspended while being transported in an electrostatic field. Alternatively, they may be film-forming materials which function to decrease the sliding friction between fibers. The use of separating agents is often desirable in overcoming the tacky or hygroscopic properties often associated with some antistatic agents. There are three classes of separating agents which have been found suitable for use in coating the synthetic fibers employed in the invention. The first type comprises inorganic particles such as silica, magnesium oxide, aluminum oxide, talc and the like, which are described more fully in Ewing, U.S. Patent 2,805,959. The second class of separating agents found suitable are lubricants and free-flowing powders such as the metallic stearates, including magnesium stearate and aluminum stearate. The third class of suitable separating agents comprises water soluble compounds and polymeric waxes, such as cationic fatty acid amide derivatives, long chain alkyl amines such as octadecyl amine, condensation products of 40 to 90% by weight ethylene oxide with higher alkyl phenols, e.g. nonyl phenol, or with tall oil fatty acids. The separating agents can be applied in the form of powders, solutions or dispersions to the fibers. These agents are advantageously added to the fibers during the crimp inhibition step; that is, by wetting the tautly held fibers therewith followed by drying in the taut condition and cutting the short fiber lengths. Certain of the wax-like separating agents, e.g. octadecylamine, which envelop the fibers with a film coating are also capable of functioning as a weighting agent, i.e. to prevent premature crimp. The amount of separating agent provided on the surface of the fibers should be between about 0.05 and 15%.

50 In general the two types of known methods which may be used for propelling flock against a backing material are (1) the use of an electrostatic field and (2) the use of a beater device. Both are well suited to the practice of the invention although the method involving the use 55 of an electrostatic field is especially preferred. When using an electrostatic field for propelling the synthetic fibers, it is highly desirable to apply to the fibers before flocking not only an antistatic agent but also a separating agent.

60 If it is desired to use electrostatic flocking for propelling the fibers to a backing, the suitably conditioned and treated short flock fibers may be distributed by means of a revolving brush or shaking device from a bin over a grid electrode charged with 10,000 to 100,000 volts. At some distance from the grid there is a metal plate connected to the oppositely charged terminal of the high voltage supply. On this plate rests a backing material covered with a thin adhesive layer. The charged flock is projected toward the ground and impinges upon the adhesive surface in a direction which is generally perpendicular to the backing material. Using this procedure it is possible to make pile fabrics having pile densities as high as 10 pounds per cubic foot and as low as 1 pound per 75 cubic foot.

Normally the flock fibers employed will have a denier ranging from about 3 to 30. As is well known in the flocking art, it is necessary to prepare the flock fibers by careful cutting techniques so that both ends are squared off perpendicular to the fiber length to provide cut ends that are clean, not frayed, and do not have stray fibrous hairs as a result of poor cutting.

If it is desired to use a beater device for propelling the treated flock fibers to the backing material, the following description provides a suitable method for practicing this aspect of the invention. Suitably treated and cut flock fibers are placed in a shaking, sieving device provided with a shaking or brushing mechanism to assure uniform deposition of fibers onto a uniformly moving backing fabric traveling below the flock supply device. The backing is supported by a heavy "belt" which passes over a block rotating at a speed such that the corners of the block set up a uniform rapid vibration on the belt. This causes the fibers to stand on end and become embedded in an adhesive spread upon the backing prior to deposition of the flock fibers. Subsequently, vacuum devices are utilized to remove non-adhering flock from the adhering fibers. The excess flock so obtained is recycled by pneumatic devices to the supply chamber.

Any suitable backing material may be used as a base or substrate for receiving the propelled flock fibers. The backing material may be a woven, knitted, or non-woven fabric, or may be a film such as cellophane, polyethylene film, or polyester film. The backing material should be coated with a thin layer of suitable adhesive which will remain at least tacky during the flocking operation and which can be solidified after propelling the flocked fibers to the backing. The adhesive may be solidified by cooling or air drying, or the adhesive may be selected to be a thermosetting adhesive in which case it may be cured to a solid condition by heat and/or catalysts. Typical adhesives include solutions or dispersions of rubber, polyvinyl acetate, polyurethanes, etc.

After the flocked fibers have been deposited on the backing material, the resulting pile fabric must be subjected to conditions such that the latent crimp is developed. These conditions may be applied to the pile fabric, if carefully controlled, simultaneously with the solidification of the adhesive. Often, however, it is more desirable to first solidify or set the adhesive and then separately treat the pile fabric to develop the crimp. Depending upon the choice of synthetic fiber and upon the nature of the desired crimp, a variety of known conditions can be employed to develop the latent crimp in the pile fibers which are attached to the backing material. Suitable techniques for the described types of fibers include heat treatment alone, e.g. by hot air blasts, hot water or steam. For certain types of fibers chemical shrinking agents can be used to advantage to develop the latent crimp. For the above mentioned two-component acrylonitrile polymer fibers which are especially suitable in practicing the invention, the latent crimp is preferably developed by treating the pile fabric under hot wet conditions. Often it is entirely practical to develop the crimp in the pile fabric conjointly with a dyeing or finishing operation, e.g. during which the fabric is subjected to a hot dye bath or to hot and/or wet finishing conditions. If a chemical shrinking agent is used or if other wet conditions are used to develop the crimp, it will be later necessary to dry the pile fabric.

One of the primary advantages of the invention resides in the provision of a rapid, economical process for preparing flocked fabrics composed of synthetic organic polymeric pile fibers. Another important advantage is that the process provides a means for preparing flocked fabrics which have certain properties which are superior to the flocked fabrics containing straight or uncrimped pile fibers. The property advantages of the products made in accordance with the invention include improved aesthetics, more pleasing hand, less "bristly" fabrics, more wool-like

texture, greater cover and bulk, and greater insulating capacity. Another advantage of the present invention is that it readily affords a great number of styling variations in the resultant pile fabrics.

The present invention may be used to prepare flocked pile fabrics which have a wide variety of uses, for example, suedes, velvets, furs, floor covering materials, such as carpets and tiles, blankets, insulating facing cloths, apparel interliners, and various laminated multi-layer fabrics. One example of a laminated fabric which can be prepared in accordance with the invention comprises a backing material to which is attached a flocked pile layer and finally a top cloth which is adhered by means of an adhesive to the surface of the pile. This type of structure is especially suitable as an insulation lining for wearing apparel. Another example of a suitable laminated fabric is one in which an adhesive is applied to the bottom surface of a backing material containing on the opposite surface a flocked pile layer as produced by the invention. Following the application of a support cloth to the adhesive a layer of straight, non-latently crimpable flock is applied to the adhesive such that the fibers of the second pile layer are perpendicular to the support cloth. Optionally, another backing material might then be applied by means of an adhesive to the exposed surface of the straight flocked pile. An additional example of a laminated fabric involves the application of a separate layer of flocked latently crimpable fibers to each side of a backing cloth, followed by development of the crimp. A double faced article of such a structure is especially suited to the formation of blankets. A modification of such a double faced article involves using as the inner layer or support a sandwich type structure composed of a third pile layer of straight, non-latently crimpable flocked fibers between two sheets of support cloths. A wide variety of such structural modifications will be apparent.

The flocked pile fabrics of the invention can also be advantageously used to prepare tufted fabrics, e.g. by passing the tufting threads through the flocked pile layer and into attachment with the backing. In this way the flocked pile layer forms a background for the tufts so as to offer pleasing aesthetics and permit a reduction in the quantity of tufts needed for suitable cover and compressional resilience.

It has been found that a unique structure offering unusual functional and aesthetic properties can be achieved by the above described flocking process. This unique structure can be best understood by examining individual fibers in the layer. Thus as illustrated schematically in FIGURE 1, a typical fiber as viewed from the side (disregarding any region extending below the adhesive line) would be found to have a relatively straight part and a curved part. If the fiber was bisected to produce two sections or halves of equal length, i.e. each equal to one-half the extended fiber length AB, it would be seen that the curved part is confined essentially to the upper section or AE. If one then imagines a plurality of such fibers all adhered in upstanding relationship with respect to a common base, the effect would be to create two superposed layers or portions, each coextensive with the adhesive layer. In the upper portion the fibers sections would all be crimped and bent over. Moreover, because the fiber ends in that top portion would extend randomly in many directions, this being necessary for suitable compressional properties, numerous fiber-to-fiber entanglements would appear. On the other hand, fiber sections in the lower or support portion, i.e. immediately adjacent the adhesive layer, would be generally straight, or free of crimp, spaced apart, parallel, and, of course, essentially perpendicular to the base. Although these two portions of the pile would contain equal weights of fiber, the lower would be of greater thickness but of considerably less pile density. The unique nature of this pile configuration is illustrated in FIGURE 2 which shows schematically the

representation of fibers in a sample of a product of the invention.

It is a surprising and highly advantageous feature of the products of the invention that maximum bulk is achieved at a comparatively low crimp frequency. Thus as shown in FIGURE 3, at a load of 3.1 p.s.i. a pile layer attains a maximum bulk at 2 crimps per inch (c.p.i.). Normally, the crimped portion of the fibers will have an average crimp frequency of 1 to 8 c.p.i. to give a suitably high bulk, e.g. of at least 10 cc./gram at 3.1 p.s.i. load. These findings in connection with the products of the invention are in marked contrast to the prior art where heretofore it had been found that the higher the crimp frequency of a fiber, the greater will be the bulk of a pile fabric produced therefrom.

Referring once again to FIGURE 1, the ratio of the extended fiber length AB to the effective length of the crimped fiber CB is defined as a constant K. The radius of curvature of a circle drawn using the major arc or curved surface of the crimped section of the fiber is designated as  $r$ , which is equal to the distance CD in the relaxed state. The angle P is the angle subtending the arc of the circle forming a curved part of the crimped section of the fiber. The circumference  $c$  in inches is the circumference of the circle whose radius of curvature is  $r$  such that  $c$  equals  $2\pi r$ . Also the crimp frequency in crimps per inch of the fiber is simply the reciprocal of the circumference of the circle having a radius of curvature  $r$ . Hence, the ratio CD/DB may be defined as the ratio of the radius of curvature of the uncrimped section of the fiber to the length of the uncrimped portion of the fiber when relaxed. The pile fabrics of the invention will preferably have a K value in the range of 1.1 to 1.7, a ratio CD/DB between 0.95 and 0.15, and the upper 50% portion of the pile will have a pile density at least 1.5 times that of the lower 50% portion.

The high resistance to compression provided by the products of the invention arises owing to the optimum frequency of the crimp and to the confinement of that crimp in the upper portion of the pile layer. Thus straight pile fibers (no crimp) in a fabric are acted upon individually, hence buckle rapidly under compressive forces. As the crimp level of a fiber of given length increases, e.g. at 2 c.p.i. as illustrated in FIGURE 3 in connection with  $\frac{1}{4}$ -inch flock of 20 denier, there develop two structural factors important to resistance to buckling. The first of these is the decreased slenderness (shorter hence more rigid nature) of the supporting columns and the manner in which the ends are essentially permanently fixed (one end in adhesive, the other by fiber-to-fiber entanglements). Secondly, the crimped fiber sections in the upper portion of the pile layer become entangled to form a high density matrix which distributes stress laterally in absorbing loading energy. When the crimp frequency becomes excessively high, the supporting sections of the fibers become buckled, as a result the density of the upper and lower portions become nearly equal and, since support will be then derived mainly from interfiber friction at the fiber contact points, overall bulk is reduced. It will be understood from the above that the optimum bulk to be developed in a sample will depend upon the radius of curvature of the major arc of the crimp, the extended fiber length, and of course the ratio CD/DB.

Although the novel pile fabrics of the invention have been described especially in connection with a flocking process, it is to be understood that other methods may be used for their preparation.

The following tests are used in connection with the novel products of the invention.

#### Measurement of crimp frequency

Pile fibers in a fabric are sheared off at the glue line, distributed over a glass plate and photographed. Twenty-

five fibers were examined at random measuring the radius of a circle drawn through the major curvature of the fiber. The crimp frequency (c.p.i.) was calculated using the equation:

$$c.p.i. = \frac{1}{2\pi r}$$

with the value used for  $r$  being the average radius for the fibers so examined.

#### Pile fabric compression test

Specimens measuring 4" x 4" are taken from pile fabric samples to be tested. Two specimens are normally taken from each sample and the data reported are the average of results from both. The specimens are conditioned in two steps according to common textile testing procedures wherein a pre-conditioning at  $130^\circ \pm 10^\circ$  F. in moving air from a minimum of two hours is followed by a final conditioning at 65% RH and 70° F. in moving air for a minimum of sixteen hours. The conditioned specimens are weighed to the nearest 0.01 gram and measured to the nearest 0.02 inch taking an average of three measurements in both length and width.

Each specimen mounted on a compression cell is subjected to compression with pile side up at the rate of 0.2 inch/minute on an Instron Tester using a circular presser foot of 10 in.<sup>2</sup>.

The load cycling controls of the tester are set so as to cause the crosshead to return when the desired full load has been applied. In the case of carpets of high denier fiber (12-25 d.p.f.), a maximum load of 10 p.s.i. is used; whereas for fleeces and lower denier fiber (2-12 d.p.f.), the maximum load is 1.1 p.s.i. The crosshead stops when the pressure has returned to zero. After a two minute interval a second compression cycle is run in the same manner. Following the second cycle of compression and unloading, the specimen is taken from the tester and the pile is sheared off as evenly and cleanly as possible from the surface of the adhesive using heavy duty barber clippers equipped with a No. 000 (fine) clipper head. The sheared backing is then weighted to the nearest 0.1 gram. The sheared backing is subjected to compression testing in the same manner as in the un-sheared form except that it is loaded at a rate of 0.1 inch/minute crosshead speed. During the compression test the stress is recorded and appears on the chart as a pen line whose coordinates are stress in lbs. and separation between cell and presser foot in inches. From this graphic data, specific points can be extracted. On the first compression cycle, a specific point of interest is the cell presser foot separation when the presser foot barely touches the sample and the pressure starts to increase. This separation is used as the initial thickness of the specimen. From this second cycle and its record, the integrator count for the load portion of the cycle is obtained.

#### Specific volume or bulk

The specific volume or bulk of the pile layer at given load is calculated as the volume of the pile at the given load divided by the pile weight. The pile volume at the given load is determined from the second compression cycle as the difference between the thickness of the pile fabric and the backing at the given load times the specimen area, suitable conversion factors being applied.

The following examples illustrate specific embodiments of this invention without intending to limit the scope of the invention. All parts are expressed by weight unless otherwise indicated.

#### EXAMPLE I

A continuous filament yarn (1000 denier, 140 filaments) was spun from bicomponent filaments (100% acrylonitrile polymer and 95% acrylonitrile/5% sodium styrene sulfonate copolymer) in accordance with Taylor

U.S. 3,038,237. The yarn was wrapped on a metal frame so that the ends of the yarn were taut on the frame. A total of 32 grams of the yarn, which in relaxed condition would give a boil-off spontaneous crimp of 13 crimps per inch and a crimp index of 25%, was then treated at the boil in a bath made up as follows:

|                                   |     |       |
|-----------------------------------|-----|-------|
| Water                             | ml. | 1280  |
| Antistatic agent "A" <sup>1</sup> | g.  | 0.16  |
| Sodium sulfate                    | g.  | 3.20  |
| Antistatic agent "B" <sup>2</sup> | g.  | 1.28  |
| Acetic acid                       | g.  | 0.16  |
| Malachite green dye               | g.  | 0.256 |
| Red dye <sup>3</sup>              | g.  | 0.672 |

<sup>1</sup> Aqueous solution containing 10% 2-methyl-2,4-pentane diol and 60% condensation product of oleyl alcohol and ethylene oxide (1:20 mol ratio).

<sup>2</sup> C<sub>12</sub>-C<sub>18</sub> fatty alcohol plus cetyl trimethyl ammonium bromide (50/50).

<sup>3</sup> [2-(p-[2-chloro-4-nitrophenylazo]-N-ethylanilino)ethyl] trimethylammonium chloride.

After one and one-half hours at the boil, the temperature was then lowered to 80° C. and there was added 4.8 g. of a separating agent comprising a cationic fatty acid amide derivative ("Ceranine HC"). The frame was removed from the bath and without rinsing the fibers were allowed to dry in the taut condition. The frame and its dyed fibers were then submitted to dry heat at 130° C. for 10 minutes, thus setting the fiber in a straight condition. The fiber was then removed from the frame and cut by means of a paper cutter into flock  $\frac{1}{8}$ -inch in length. To facilitate the cutting the straight fibers were laid between layers of cardboard and trapped as a sandwich, the cardboard being removed after each cut through a layer of fibers.

The flock so prepared was free-running and had no tendency to clump upon shaking in a container. The flock was allowed to stand at room conditions in an uncovered container overnight. The flock was then transferred to a Waring Blender and at low speed was fluffed or separated into a very light porous separated mass. The flock was placed in a 3 inch transparent acrylic plastic basket, approximately 4 inches long, one side of which was a  $\frac{1}{8}$ -inch mesh metal screen which served as a positive electrode of an 18,000 volt electrostatic generator. The negative electrode was a metal plate which also was the ground potential. A scrim fabric (4 oz./yd.<sup>2</sup> cotton muslin) was coated with a thin coating of a polyurethane resin adhesive and placed in an oven for a few minutes to dry. A second coat of the same adhesive was then applied and while still wet the scrim fabric was placed on the ground plate. The flocking cage was then shaken in such a manner to allow the flock to fall onto the adhesive surface at a potential of 18,000 volts. This was continued until an additional shaking did not produce any further increase in pile density. The scrim fabric was then removed and placed in an oven at 90° C. for about 1/2-hour to cure the adhesive. The excess flock was removed and the fabric was then treated with atmospheric steam for a short time to develop the crimp of the bicomponent fiber. By comparison to unsteam-treated flock it was evident that a very dense curly, bulky structure was obtained via the steaming treatment, quite different from the normal straight chenille-type pile structure otherwise obtained with non-latently crimpable flock. By coating the opposite side of a previously flocked surface, a second side could then be flocked with the same self-crimping bicomponent fiber to give a good blanket-like fabric approximately  $\frac{1}{8}$ -inch in thickness after steaming.

#### EXAMPLE II

A 2,000 denier, 200 filament, drawn yarn from the same bicomponent filaments as used in Example I, was wound on a frame in the same manner as in Example I, and treated at the boil in a bath made according to the same formula as in Example I. However, after heat setting, this fiber was cut on a guillotine-type paper cutter

to  $\frac{1}{16}$ -inch length material. A fabric prepared according to the same procedure as used in the earlier example was then made but in this case a higher voltage, approximately 20,000-38,000 volts was used. After achieving the highest possible density as could be obtained by repeatedly shaking the container holding the straight flock over the adhesive scrim fabric, the fabric was allowed to dry and thereafter exposed to atmospheric steam. The resulting fabric had a thickness of approximately 0.122 inch of which approximately 0.10 inch was due to the bulked fiber flock on the surface. Then a similar fabric was prepared using a tarred backing fabric, the density of the pile prior to steaming being 2.37 pounds/cu. ft. at a height of 0.240 inch. After steaming the pile height became 0.12 inch and the density increased to 4.45 pounds/cu. ft. The fabric exhibited a dense resilient surface resembling a fine mohair furniture upholstery covering and was suitable for a rug, blanket or upholstery fabric.

#### EXAMPLE III

A bicomponent polyester fiber was prepared by the co-spinning side-by-side of high and low shrinkage members, 40:60 percent ratio. Respectively these members were a random copolymer of ethylene terephthalate/ethylene hexahydroterephthalate (83/17 mol percent ratio) and a random copolymer of ethylene terephthalate/ethylene 5-(sodium sulfo)-isophthalate (98/2 mol percent ratio). The denier of the filamentary composite was 2.2 d.p.f.

Twenty grams of the composite filaments in the form of a 720 denier tow was wrapped tautly on a steel frame and treated at 40° C. with the following solution for one hour:

|                                     |     |      |
|-------------------------------------|-----|------|
| Water                               | ml. | 3520 |
| Antistatic agent "A" (of Example I) | g.  | 0.4  |
| Antistatic agent "B" (of Example I) | g.  | 3.2  |
| Sodium sulfate                      | g.  | 8.0  |
| Acetic acid                         | g.  | 0.4  |
| Separating agent (of Example I)     | g.  | 12.0 |

The fiber was then air dried while taut on the frame, unwound, and then cut into  $\frac{1}{8}$ " lengths using a guillotine cutter. The flock was then placed in a Waring Blender with 2.5% of "Alon C" (Al<sub>2</sub>O<sub>3</sub>) and mixed thoroughly. This coating provided for easy fiber separation in the flocking process. The fiber was then placed in an electrostatic flocking device as described in Example I and shaken onto a cotton scrim fabric previously coated with a 10-mil layer of a polyurethane adhesive to achieve a pile density corresponding to 1.25 lbs. per cu. ft. The flocked fabric was placed in an oven at 130° C. to cure the adhesive. Atmospheric steam was played upon the pile surface of the fabric for one minute and a soft, crimped surface texture was obtained. The fabric was useful as a blanket, as an insulating liner for jackets, and in bed-spreads or upholstery fabrics. The performance of fabrics composed of fibers crimped in this manner is particularly notable because (1) high "cover" is achieved with a minimum of fiber content, and (2) warmth is achieved in a light weight fabric. As an example of case (1), the appearance of the fabric prior to crimp development was "lean"; that is, the fibers were observed as individuals and provided a minimum of cover owing to their perpendicular orientation with respect to the surface. After crimping, however, the fibers became intimately associated with one another developing continuity in the pile surface to provide cover. The stiffness of individual fibers is considerably altered as a result of crimp development to provide a soft hand in contrast to the "bristly" hand of uncrimped fibrous pile layers.

The improved insulating value of the crimped fiber pile structure over those of straight fibers results from fiber intermingling to decrease convection, the "cells" so formed limit the circulation of air. In use, a 2-pound

## 11

blanket comprised of fabric containing post-crimped flock provides comparable warmth to a 3-pound commercial woven blanket and has an added advantage of increasing sleeping comfort because of the decreased weight.

## EXAMPLE IV

Flock of  $\frac{1}{8}$ -inch length was prepared by cutting 6-denier bicomponent filaments of the composition as described in Example I.

Ten pounds of flock so prepared was loaded into a stock dye kettle with hot water being added, simultaneously as an aid in packing the fiber tightly. A dye solution with the following composition was circulated through the stock at a temperature of 95-100° C. for one hour:

|                                     |         |     |
|-------------------------------------|---------|-----|
| Water                               | gallons | 25  |
| Red dye (of Example I)              | pounds  | 0.2 |
| Antistatic agent "A" (of Example I) | do      | 0.1 |
| Acetic acid                         | do      | 0.1 |
| Antistatic agent "B" (of Example I) | do      | 0.4 |

Following the one-hour dye treatment, the bath was allowed to cool to 60° C. and one pound of octadecylamine was added as a separating and weighting agent. After further cooling to 30° C. the excess liquor was drained off and the dyed flock was dried in a tumble dryer at 105° C. The flock particles were separated by passing through a series of screens ( $\frac{1}{4}$ - $\frac{1}{8}$ " mesh). At this stage the particles had a waxlike coating which served to restrain premature crimp development which would otherwise occur on drying. The flock was then placed in an electrostatic flock applicator charged to 20,000 volts. The applicator was shaken to discharge the flock through its screen aperture onto a previously prepared cotton scrim whose surface was coated with a 10-mil layer of polyurethane adhesive solution. The flock was thus directed to form a pile layer having a density of 1.5 oz./yd.<sup>2</sup>. The fabric was then dried at 130° C. for one-half hour to cure the adhesive. In this state, the pile fibers were straight and oriented perpendicularly to the scrim backing. In order to produce a fabric of pleasing hand as desired for apparel use, the fabric was rinsed in warm water, 50° C., to remove the crimp restraining waxlike coating. The fabric was then dried at 70° C., whereupon the crimp of the two-component fiber developed and the desired soft hand was achieved. The fabric was well suited for the manufacture of insulating liners for jackets, baby blankets, and upholstery fabrics.

## EXAMPLE V

A tow of 20 denier continuous filaments was spun from a bicomponent composition of 100% acrylonitrile polymer on one side of the filament and 96% acrylonitrile/4% sodium styrene sulfonate copolymer on the other side of the filament in accordance with Taylor U.S. 3,038,237. The tow was wrapped on a frame so

| Example | Fiber Denier | Fiber Length (in.) | Pile Density (lbs./ft. <sup>2</sup> ) | Crimp Frequency, c.p.i. | Pile Bulk (cc./g. at 3.1 p.s.i.) | Work to Compress to 10 p.s.i. (in.-lbs./in. <sup>2</sup> ) |
|---------|--------------|--------------------|---------------------------------------|-------------------------|----------------------------------|------------------------------------------------------------|
| VI      | 10           | .23                | 2.8                                   | 1.8                     | 16.9                             | .643                                                       |
| VII     | 20           | .25                | 3.0                                   | 7.6                     | 12.0                             | .397                                                       |
| VIII    | 10           | .23                | 2.4                                   | 9.4                     | 10.3                             | .544                                                       |

that the ends of the filaments were held taut while the tow was passed through a bath of a 4% by weight aqueous solution of cetyl pyridinium chloride. Excess solution was squeezed from the tow by passage through nip rolls and the tow was dried at 80° C. The filaments contained 1% by weight, based on the weight of the fibers, of cetyl pyridinium chloride. The dried tow was then cut into flock particles 6 millimeters in length. The cut fiber was then flocked by electrostatic means as described in Example I onto a cotton fabric coated with an

## 12

acrylic polymer adhesive to yield a flocked fabric having a pile fiber density of 6.5 ounces per square yard. The adhesive was cured at 149° C. At this stage the pile fibers had no crimp and were perpendicular along their full lengths to the adhesive line. The pile fabric was then subjected to the action of atmospheric steam for one-half minute to permit crimp development of the bi-component fiber and then dried at 71° C. for 15 minutes. The resulting fabric showed a high degree of resistance to compression and had characteristics that would make it suitable for use as a carpet. An examination of the compression characteristics through a range of 0-10 p.s.i. using Instron Compression Test for carpets showed it to have a high work-to-compress ( $W_c = .544$  in.-lb./in.<sup>2</sup>) wherein  $W_c$  is the work per unit area required to compress the carpet sample to 10 p.s.i. indicative of "bounce," and a high bulk value (15.8 cc./g. at 3.1 p.s.i.). The crimp frequency was found to be 2.4 c.p.i. Examination of the pile structure (FIGURE 1) led to the following description:

Essentially each fiber had one end fixed in the glue line from which it extended vertically for a distance of 54% of its length, then bent to define an arc subtended by an angle  $P$  of 100°. The tip-to-tip angle was 22° and the ratio of the extended fiber length to pile height (AB/BC) was 1.25. The ratio of the radius of curvature to the straight portion was 0.49. By actual count there were 8500 fibers per square inch. The distance between fiber axes averaged 0.011 in. for the 20 denier (2 mil diameter) fibers used; the curved portion of the fiber extended horizontally to cover a distance equal to that occupied by 8 fibers. The fiber density of the upper 50% of the structure was calculated to be 1.64 times that of the lower 50%. There was a density gradient within the upper 50% and the density increased toward the surface, the maximum being achieved, in the region where the horizontal component of fiber direction is greatest.

The flocked crimped fiber of this example according to FIGURE 1 had the following structural parameters: radius of curvature  $r$  is .065";  $K$  is 1.25;  $DB$  is 0.14 inch;  $CD/DB$  is 0.49; and  $DB/AB$  is 0.54.

## EXAMPLES VI-VIII

Additional flocked fabrics were prepared from the same composition of bicomponent acrylic fibers as used in Example V. The flocking conditions were varied, however, to yield products having properties as indicated in Tables I and II. Examples VI and VII illustrate the preparation of fabrics having desirable properties in accordance with this invention, whereas Example VIII illustrates the preparation of a fabric outside the scope of the invention because the crimp frequency is too high. The products of Examples VI and VII are especially suitable as paint roller covers.

TABLE I

| Fiber Parameter | Ex. VI | Ex. VII | Ex. VIII |
|-----------------|--------|---------|----------|
| $r$ (in.)       | .088   | .021    | .017     |
| $K$             | 1.14   | 1.66    | 2.1      |
| $DB$ (in.)      | .115   | 0.12    | 0.10     |
| $CD/DB$         | .76    | 0.17    | 0.17     |
| $DB/AB$         | .50    | 0.48    | 0.40     |

TABLE II

| Fiber Parameter | Ex. VI | Ex. VII | Ex. VIII |
|-----------------|--------|---------|----------|
| $r$ (in.)       | .088   | .021    | .017     |
| $K$             | 1.14   | 1.66    | 2.1      |
| $DB$ (in.)      | .115   | 0.12    | 0.10     |
| $CD/DB$         | .76    | 0.17    | 0.17     |
| $DB/AB$         | .50    | 0.48    | 0.40     |

In order to show the effect of different treatment conditions for developing the latent crimp in the fibers after

crimping, a series of flocked fabrics was prepared similar to that described in Example V, except that the amount of sodium styrene sulfonate content on one side of the bicomponent fiber was varied as indicated in Table III, the denier of the fiber was varied and the exposure time to atmospheric steam was varied.

TABLE III

| Fiber Denier | % Sulfonate in Copolymer | Crimp Frequency, Steam Exposure Time |                  |
|--------------|--------------------------|--------------------------------------|------------------|
|              |                          | 0.5 min.                             | 15 mins., c.p.i. |
| 3            | 4                        | 4.0                                  | 12               |
| 6            | 4                        | 3.5                                  | 10               |
| 10           | 4                        | 3                                    | 9                |
| 20           | 2                        | *0.5                                 | 2.4              |
| 20           | 4                        | 2.4                                  | 7.5              |
| 30           | 4                        | 1.5                                  | 5                |

\* Less than 10 cc./g. bulk.

It will be understood that all of the flock fibers need not have a latent capacity to crimp. In fact for pile fabrics to be used for certain applications up to 75% by weight of the flocking fibers can be advantageously provided by straight fibers which have no latent capacity to crimp. The amount of noncrimpable fibers will, of course, depend upon the nature of the end use.

What is claimed is:

1. Method for the manufacture of pile fabrics comprising the steps of providing a plurality of short straight, latently crimpable synthetic organic polymeric fibers which have been treated to temporarily inhibit premature crimp, depositing the thusly treated fibers upon an adhesive coated backing material to provide a pile layer of upstanding fibers thereon, and treating the resultant fabric to develop the latent crimpability of the fibers.

2. Method of claim 1 wherein said fibers are electrostatically deposited upon said adhesive coated backing member.

3. Method of claim 1 wherein the fibers are treated with a separating agent prior to deposition upon the said adhesive coated backing material.

4. Method of claim 1 wherein said treatment to temporarily inhibit premature crimp comprises holding long fibers tautly in the longitudinal direction while wetting with a separating agent, drying the treated fibers in taut condition and cutting short fiber lengths therefrom.

5. Method of claim 1 wherein the fibers are treated with an antistatic agent prior to deposition upon the said adhesive coated backing material.

6. Method of claim 1 wherein the latent crimpability of the fibers is developed by hot wet processing conditions.

7. Method of claim 1 wherein the said fibers are multi-component fibers.

8. Method of claim 7 wherein the said multi-component fibers have at least two components wherein each is composed of an acrylonitrile polymer.

9. Method of claim 7 wherein the said multi-component fibers have at least two components wherein each is composed of a polyester.

10. A pile fabric comprising a plurality of short synthetic organic polymeric fibers individually and randomly attached in generally upstanding relationship to an adhesive layer, the pile formed of said fibers comprising a support portion occupied by the lower 50% sections of the extended length of said fibers and an upper portion occupied by the remaining 50% sections of the extended length of said fibers, fiber sections in said support portion being essentially spaced apart, free of crimp, and perpendicularly aligned with respect to said adhesive layer, fiber sections in said upper portion having an average crimp frequency of 1 to 8 crimps per inch thereby creating a pile surface having a random and multidirectional array of fiber sections and fiber-to-fiber entanglements.

11. Fabric of claim 10 wherein said fibers are multi-component fibers.

12. Fabric of claim 11 wherein the said multi-component fibers have at least two components wherein each is composed of an acrylonitrile polymer.

13. A pile fabric comprising a plurality of short synthetic organic polymeric fibers bonded at their base to an adhesive layer, half of the extended length of individual fibers having an average crimp frequency of 1 to 8 crimps per inch and said halves together constituting the upper portion of said pile, the remaining halves of individual fibers being substantially straight and constituting the support section of said pile, the fibers being in generally multidirectional entangled arrangement in said upper portion and in generally parallel spaced apart relation in said support portion, the pile density in said upper portion being at least 1.5 times the fiber density in said support portion.

14. Fabric of claim 13 wherein said fibers are of essentially uniform extended length, said length being about 0.1 to 0.35 inch.

15. Fabric of claim 13 wherein said fibers have a ratio CD/DB between 0.95 to 0.15 wherein CD is the radius of curvature of said halves of said individual fibers constituting said upper port of said pile, and wherein DB is the length of said remaining substantially straight halves of individual fibers constituting said support section of said pile.

16. Fabric of claim 13 wherein said fibers have a K value defined by the ratio AB/CB in the range of 1.1 to 1.7 wherein AB is said extended length of said short fibers, and wherein CB is the effective length of said short fibers in crimped form.

#### References Cited by the Examiner

#### UNITED STATES PATENTS

|              |        |              |           |
|--------------|--------|--------------|-----------|
| 2,439,815    | 4/1948 | Sisson       | 161—177   |
| 2,776,223    | 1/1957 | Brown et al. | 117—17    |
| 55 3,024,518 | 3/1962 | Newton       | 161—66 X  |
| 3,038,235    | 6/1962 | Zimmerman    | 161—177 X |
| 3,038,237    | 6/1962 | Taylor       | 161—177 X |
| 3,203,821    | 8/1965 | Domin        | 117—17    |

ALEXANDER WYMAN, Primary Examiner.

EARL M. BERGERT, R. H. CRISS,

Assistant Examiners.